

W. M. FULTON.

PROCESS FOR THE MANUFACTURE OF FLEXIBLE CORRUGATED WALLS.

APPLICATION FILED OCT. 8, 1914.

1,192,412.

Patented July 25, 1916.

*Fig. 1.*



*Fig. 2.*



*Fig. 3.*



Inventor

Winton M. Fulton.

By  
H. W. Cameron, Lewis & Associates  
Attorneys

# UNITED STATES PATENT OFFICE.

WESTON M. FULTON, OF KNOXVILLE, TENNESSEE, ASSIGNOR TO THE FULTON COMPANY, OF KNOXVILLE, TENNESSEE, A CORPORATION OF MAINE.

## PROCESS FOR THE MANUFACTURE OF FLEXIBLE CORRUGATED WALLS.

1,192,412.

Specification of Letters Patent. Patented July 25, 1916.

Application filed October 8, 1914. Serial No. 865,748.

*To all whom it may concern:*

Be it known that I, WESTON M. FULTON, a citizen of the United States of America, and a resident of Knoxville, Tennessee, have 5 invented a new and useful Improvement in Processes for the Manufacture of Flexible Corrugated Walls, which invention is fully set forth in the following specification.

This invention relates to methods of making 10 expandable and contractible corrugated vessels, and more particularly to making the tubular walls of such vessels whereby they will possess great flexibility combined with durability.

15 Heretofore walls for flexible corrugated vessels have been made from die-drawn seamless metal tubes and such a method is described in my U. S. Patent No. 975,519. As pointed out in that patent, the operation 20 of die-drawing the seamless metal tube results in hardening the surfaces of the tubular walls by increasing the density of the metal at and near the surface while leaving a less dense interior portion of metal between the 25 hardened surfaces. A stratification of the metal in the walls of the tube results, and when the tube is corrugated to give its flexibility the corrugations possess layers of metal differing in physical characteristics 30 such as hardness, elasticity, and other properties. Vibratory movements of the walls are accompanied by more or less bending back and forth at the bends of the corrugations with displacements of the layers 35 which finally yield to these strains and crack, thereby terminating the life of the vessel. In my said patent there is also pointed out the desirability of making the flexible corrugated wall of uniform molecular structure 40 and consequently of uniform hardness, toughness and elasticity throughout its cross-section, and there is described therein one method of making such a wall by removing from its surface the outer hardened 45 layers.

I have discovered that a uniform molecular condition can be produced in metal, such as steel, copper, brass or the like, without removing these outer layers, by starting 50 with a thicker sheet or wall than is desired in the finished product and working the metal into a thin sheet or wall, the thinness of which varies for different metals. When the metal has reached the proper thinness, 55 it is found by examination of photomicro-

graphic sections of the wall that the less dense central portion has disappeared from between the condensed surface layers and that the condition of the metal as to density, 60 hardness and elasticity is substantially uniform throughout. For example, in the case of soft low brass which I may use for making the walls of my flexible corrugated tubular vessels, a thickness of about .008 of an inch is sufficient for reducing the metal to 65 practically uniform molecular condition in the respects noted. My invention which is based on this discovery is capable of expression in a variety of ways or methods of procedure, one of which, for the purpose of 70 illustration, is herein specifically described; but the method thus described is given solely for the purpose of illustrating the invention and not for defining the limits thereof, reference being had to the appended claim for 75 that purpose.

With a view of assisting the description, reference is had to the accompanying drawings, in which:—

Figure 1 is a transverse sectional view 80 through a die-drawn seamless metal tube used as a blank showing the stratified condition of the walls in magnified cross-section; Fig. 2 shows the same tube with the outer layers merged into each other; and 85 Fig. 3 is a longitudinal sectional view highly magnified showing a collapsible and extensible wall embodying my improvement.

I take a seamless drawn tube such as 90 illustrated in Fig. 1, in magnified cross-section, preferably of soft low brass, and of a diameter suitable to make a corrugated collapsible and extensible wall of the desired dimensions, and subject the tube to repeated drawing operations between a mandrel and 95 a die until the intermediate layer 1 vanishes or until the outer dense layers 2 and 3 merge together into one layer 4 practically homogeneous in cross-section, as can be determined by microscopic examination. For 100 this particular material this condition will be secured when the wall is reduced to approximately .008 of an inch in thickness. The tube is then corrugated in the customary manner. Such a corrugated tube is shown 105 by way of example in Fig. 3. Should it be desired to produce a wall capable of withstanding considerable pressure, the wall may be laminated in the manner described in my U. S. Patent No. 979,460. The laminated 110

wall will give the desired strength and possess uniform density without sacrificing flexibility to an extent sufficient to detract from its efficiency.

5. What is claimed is:—

The process of making expandible and contractible corrugated tubular walls consisting in subjecting a seamless metal tube having thin walls to a drawing operation to

10 work the metal of the denser surface layers into each other and produce uniform density

in the wall, and then corrugating the wall to render the same expandible and contractible.

In testimony whereof I have signed this 15 specification in the presence of two subscribing witnesses.

WESTON M. FULTON.

Witnesses:

H. T. PATTON,  
H. S. McCoy.